

# UNITED STATES PATENT OFFICE.

LOUIS S. ROSS, OF NEWTONVILLE, MASSACHUSETTS, ASSIGNOR TO CENTRAL RAILWAY SIGNAL COMPANY, OF PITTSBURGH, PENNSYLVANIA, A CORPORATION OF NEW JERSEY.

## COMPOSITION FOR RAILWAY SIGNAL TORPEDOES.

1,404,653.

Specification of Letters Patent. Patented Jan. 24, 1922.

No Drawing.

Application filed October 7, 1920. Serial No. 415,264.

To all whom it may concern:

Be it known that I, Louis S. Ross, a citizen of the United States, residing at Newtonville, in the county of Middlesex and State of Massachusetts, have invented certain new and useful Improvements in Compositions for Railway Signal Torpedoes, of which the following is a specification.

This invention relates to improvements in compositions for railway signal torpedoes, and is for use in torpedoes that are suitably attached to the head of a railroad rail to be exploded by the wheel of the locomotive for giving a signal to the engineer, as is well understood by those skilled in this art.

It is well-known to those skilled in this art that the explosive for railway signal torpedoes is made either in the form of a loose powder or a molded tablet, and my improved composition is adapted to be used in either of the above forms, or partly tablet and partly loose powder, as will be pointed out hereinafter.

The primary objects of my improved composition for railway signal torpedoes are—

1. To produce a louder detonation for a given quantity of composition, whereby the amount of composition used may be reduced, thus effecting economy in the manufacture, and at the same time to enable a smaller torpedo to be used, which among other advantages, is less liable to be pushed from the track, by the locomotive wheel than a larger torpedo, and would be of value to the trainmen because of the reduced size, enabling a greater number to be carried in a given space.

2. To add to the safety in the manufacture of the composition while eliminating the sensitiveness of previous torpedo compositions to friction and spontaneous ignition, which are present in the torpedo compositions now in use.

3. To produce a railway signal torpedo composition, which adds a signal flash to the signal detonation, whereby the engineer may see as well as hear the explosion of the torpedo which takes place the instant it is struck by the pilot wheels at the front end of the engine.

4. My improved composition which involves all the foregoing objects is composed of perchlorate, aluminum, sulphur, barium nitrate, sand or sharp flint, and when made in tablet form dextrine is added as a binder. If, how-

ever, the composition is to be used in powder form dextrine is omitted, and in either form of the composition the sand or flint may be omitted if desired.

In practice, I have used the foregoing ingredients in substantially the following proportions:

|                     |                 |        |
|---------------------|-----------------|--------|
| Perchlorate         | 2               | parts. |
| Aluminum            | 1 $\frac{1}{2}$ | "      |
| Sulphur             | 1               | "      |
| Barium nitrate      | 1               | "      |
| Sand or sharp flint | 1               | "      |
| Dextrine            | 1               | "      |

The foregoing proportions of the several parts may be widely varied either way without departing from the spirit and scope of my present invention.

The foregoing composition can be made to give a more brilliant flash, but at somewhat more expense, by the addition of magnesium, and also magnesium can be substituted entirely for the aluminum.

This composition may be manufactured as a moulded plastic without the aluminum or magnesium, or both, and then the desired amount of either aluminum or magnesium, or both, added as a loose binder in the case or envelope containing the explosive composition.

Furthermore, barium nitrate may be omitted, but I find that better results are obtained by its use than without it.

The perchlorate adds to the safety of the manufacture of the torpedo and safety in the storage of the torpedoes and at the same time adds to the sharpness of its detonation.

The function of the aluminum or magnesium, or both, is primarily twofold. One to furnish a flash and the other to cause a thermite reaction, causing a violent combination with the oxygen of the composition, thus adding to the violence of the detonation. The aluminum or magnesium, or both, rapidly extracts the oxygen from the other chemicals of the compound so that the violence of their action adds to the sharpness and loudness of the detonation.

It may be added here that the perchlorate in this composition increases the thermite effect, and thereby adds also to the sharpness and violence of the detonation.

The barium in this composition not only imparts insensitiveness, but also furnishes

additional oxygen to be extracted by the aluminum or magnesium, or both. It allows the last-mentioned chemicals to do more work by rapid extraction of the oxygen, and 5 this adds to the flash as well as the detonation.

Aluminum, I find, is a better extractor 10 of oxygen than magnesium, and it is also cheaper and, therefore, under ordinary conditions, preferable to the use of magnesium.

I desire it to be understood that where a 15 flash is not desired the aluminum, or magnesium, or both, may be omitted from the composition, and in this event, the remaining 20 ingredients produce a composition having the advantages of louder detonation and safety in manufacture and storage as compared with the compositions heretofore used.

Having thus described my invention, what 25 I claim and desire to secure by Letters Patent is:

1. An improved explosive composition for 30 railway signal torpedoes, comprising sulphur one part, perchlorate two parts, all 35 combined in substantially the proportions specified for producing a torpedo with in-

creased detonation and not subject to spontaneous ignition.

2. An improved explosive composition for 30 railway signal torpedoes, comprising sulphur one part, aluminum and perchlorate three and three-fourths parts, combined in substantially the proportions specified, producing a sharp flash detonation, and a composition which is not subject to spontaneous 35 ignition.

3. An improved explosive composition for 40 railway signal torpedoes, comprising sulphur one part, aluminum one and three-fourths parts, barium nitrate one part and perchlorate two parts, combined in substantially the proportions specified, producing a composition with a sharp flash detonation and which is not subject to spontaneous 45 ignition.

4. An improved composition for railway 50 signal torpedoes, comprising a perchlorate and barium nitrate combined for the purpose described.

In testimony whereof I hereunto affix my 55 signature.

LOUIS S. ROSS.